

G. GMÜR-ZEHNDER,  
TREATMENT OF REFRACtORY METALS.  
APPLICATION FILED JAN. 15, 1915.

1,150,670.

Patented Aug. 17, 1915.  
2 SHEETS—SHEET 1.



Witness,

John N. Fisher, Jr.  
W. F. Woolard

Inventor  
Gottlieb Gmür-Zehnder  
By Edson Bros  
attorneys

G. GMÜR-ZEHNDER.  
TREATMENT OF REFRACTORY METALS.  
APPLICATION FILED JAN. 15, 1915.

1,150,670.

Patented Aug. 17, 1915.  
2 SHEETS—SHEET 2.



John H. Fisher, Jr.  
W. F. Woodard.

Inventor  
Gottlieb GMÜR-ZEHNDER  
By Edson Bros  
attorneys.

# UNITED STATES PATENT OFFICE.

GOTTLIEB GMÜR-ZEHNDER, OF AARAU, SWITZERLAND.

## TREATMENT OF REFRACtORY METALS.

1,150,670.

Specification of Letters Patent. Patented Aug. 17, 1915.

Application filed January 15, 1915. Serial No. 2,478.

To all whom it may concern:

Be it known that I, GOTTLIEB GMÜR-ZEHNDER, a citizen of the Swiss Republic, residing at Aarau, in the Republic of Switzerland, have invented certain new and useful Improvements in Treatment of Refractory Metals, of which the following is a specification.

This invention relates to the treatment of refractory metals and provides an improved process and apparatus especially but not exclusively intended for the manufacture of metallic tungsten in a form suitable for the formation of metallic lamp filaments.

15 The process is based upon my discovery that if tungsten is fused to a perfectly liquid condition and is then very rapidly cooled it will not form a coarse crystalline grain (as is the case with a tungsten alloy 20 containing even a minute proportion of other metals) but will be exceedingly fine in its granular structure and will be perfectly malleable and ductile.

My process, therefore, consists in fusing 25 tungsten (usually in the form of a powder obtained from the oxid by any of the well known processes) in an electric furnace into a perfectly liquid state and in then suddenly cooling the liquid mass. The fusion 30 and subsequent rapid cooling are preferably effected in an electric furnace of resistance type, in which the tungsten is placed in an inner receptacle heated by radiation from the inclosing walls of the resistance material 35 and clear of any direct heating by the current and the tungsten is cooled by a blast of cold compressed air admitted automatically on the opening of the furnace. It is found to be important to keep the heating current 40 away from the tungsten, as if the latter is allowed to act as a conductor the heating is of a very irregular nature and a homogeneous tungsten is not obtained. Heating by radiation is therefore employed. The 45 method of cooling is also of great importance and it is found that at the extremely high temperature of perfectly fluid tungsten (about 3000° C.) the cold air blast is the most efficient means of rapid cooling, ordinary methods of cooling by liquids being 50 unsuitable owing to the instant formation of badly conducting layers of vapor.

An electric furnace embodying my invention is shown in the accompanying drawings, in which:

Figures 1 and 2 show a typical furnace

with electrical and mechanical connections in diagrammatic form, the furnace being illustrated in closed and open positions.

*a* is a tube of graphite or hard carbon or 60 other suitable refractory material, which receives the substance *a'* that it is desired to fuse.

*b* is the inner heating tube and *c* the outer inclosing tube, both of graphite or other 65 highly refractory material possessing the necessary conductivity.

*d* and *e* are respectively the top and bottom blocks which close both ends of the tubes *b* and *c* when the furnace is closed, the tubes 70 being, in the construction illustrated, carried by the upper block *d* which can be raised or lowered to open or close the furnace.

The tubes *b* and *c* and blocks *d* and *e* may 75 all be of the same material.

When the furnace is closed current is supplied through the leads *g'*, *g*<sup>2</sup> and top and bottom blocks *d* and *e* to the two tubes *b* and *c*, which are heated by the current to 80 any temperature desired. Since the temperature of the inner surface of the outer tube *c* is substantially the same as that of the tube *b* loss of heat by radiation from the latter is almost eliminated, external losses 85 being practically confined to radiation from the outer surface of the outer tube. The outer tube also combines with any oxygen which may enter or remain in the furnace and protects the substance *a'* from oxidation. The central tube *a* and its contents 90 are soon raised by the internal radiation of heat from the inner walls of the tube *b* to practically the same temperature as that of the tube and a complete and homogeneous 95 fusing of the highly refractory metals or other bodies can be attained.

When the heating operation is complete the block *d* with the tubes *b* and *c* is raised into the position shown in Fig. 2 by means 100 of the rope or cord *h* connected to the lifting arms *f* and passing over pulleys to a counter-weight. The operation may be effected by the lever *i* forming a contact breaker or switch at *k* so that the electrical 105 circuit is broken at this point immediately the furnace begins to open.

For rapid cooling of the substance in the central tube *a* a blast of cold compressed air is provided through the elongated funnels *l* inside the external casing *m* and directed upon the tube *a* from both sides. The 110

air supply is preferably turned on automatically on opening the furnace so that the cooling action may be made extremely rapid.

- 5 In starting the operation the tube *a* is filled with the material *a'* and inserted while the furnace is open as in Fig. 2. On lowering the block *d* and tubes *b* and *c*, when the latter meet the lower block *e*, the circuit is  
10 automatically completed and the current passes through the tubes *b* and *c* until the contents of the furnace are fused or brought into the desired condition.

What I claim and desire to secure by Letters Patent of the United States is:—

1. A process for producing pure malleable and ductile tungsten, consisting in fusing the metal to a perfectly fluid state and then rapidly cooling the same.
2. A process for producing pure malleable and ductile tungsten, consisting in fusing the metal to a perfectly fluid state and then rapidly cooling the same by a blast of cold air.
3. A process for producing pure malleable and ductile tungsten, consisting in fusing the metal to a perfectly fluid state by radiant heat produced electrically, and then rapidly cooling the metal.
4. A process for producing pure malleable and ductile tungsten, consisting in fusing the metal to a perfectly fluid state by radiant heat produced electrically, and then rapidly cooling the metal by a blast of cold air.
5. An electric resistance furnace for refractory materials, comprising an inner chamber formed by walls of conducting material inclosing the substance under treatment and a surrounding chamber whose walls are separated from the inner chamber by an air space and also carry current and are heated to about the same temperature as the walls of the inner chamber.
6. In an electric resistance furnace for refractory materials, two concentric vertical current conducting tubes inclosing the material under treatment, top and bottom conducting blocks between which the tubes are mounted and means for raising the tubes to open the furnace and break the electric circuit through the tubes.
7. In an electric resistance furnace for refractory materials, an inner and an outer vertical heating tube, both tubes carrying current, top and bottom conducting pieces between which the tubes make contact, and

an inner vessel containing the material under treatment and preventing it taking any part in the conduction of the current.

60

8. In an electric resistance furnace for refractory materials, an inner vessel carrying the refractory material, an inclosing chamber formed of electrically conducting heating walls, means for opening the furnace 65 and exposing the contents and means for supplying a blast of cooling air on opening the furnace.

9. In an electric resistance furnace for refractory materials, two concentric vertical 70 current conducting tubes inclosing the material under treatment, top and bottom conducting blocks between which the tubes are mounted, means for raising the tubes to open the furnace and break the electric circuit through the tubes, and means for supplying a blast of cooling air to the heated material on raising the tubes.

75

10. In an electric resistance furnace for refractory materials, two concentric vertical 80 current conducting tubes inclosing the material under treatment, top and bottom conducting blocks between which the tubes are mounted, means for raising the tubes to open the furnace and break the electric circuit through the tubes, and air blast 85 funnels directed upon the heated material.

85

11. In an electric resistance furnace for refractory materials, two concentric vertical 90 current conducting tubes inclosing the material under treatment, a bottom conducting block on which the tubes rest, an upper conducting block to which the said tubes are fixed and means for raising the upper block and the tubes to open the furnace.

95

12. In an electric resistance furnace for refractory materials, two concentric vertical current conducting tubes inclosing the material under treatment, a bottom conducting block on which the tubes rest, an upper conducting block to which the said tubes are fixed, means for raising the upper block and the tubes to open the furnace, an external casing receiving the furnace and a plurality of air blast funnels inside the said casing 100 and directed toward the center of the furnace.

100

In testimony whereof I affix my signature in presence of two witnesses.

GOTTLIEB GMÜR-ZEHNDER.

Witnesses:

HY. WIEFLISBACH,  
SIEGFR. ANGST.